

# United States Patent Office

2,937,090

Patented May 17, 1960

1

2,937,090

## PHOTOGRAPHIC EMULSIONS SENSITIZED WITH QUATERNARY DITHIOCARBAMATES

Kenneth C. Kennard and Donald M. Burness, Rochester, N.Y., assignors to Eastman Kodak Company, Rochester, N.Y., a corporation of New Jersey

No Drawing. Application May 19, 1958  
Serial No. 735,927

4 Claims. (Cl. 96—107)

This application relates to photography and particularly to sensitizing photographic emulsions.

It is well known that silver halide emulsions may be chemically sensitized with a variety of materials in order to increase the speed and generally the gamma of the emulsion, as opposed to optical sensitization in which the optical range of sensitivity is increased. Chemical sensitization usually results either from the formation of silver sulfide on the surface of the silver halide crystal, thus increasing sensitivity, or from the formation of small amount of silver from the reduction of silver halide. Other classes of compounds, such as certain ethylene oxide condensation products and certain cationic surface-active salts increase sensitivity of silver halides without apparently entering into chemical combination with the silver halide.

Carroll U.S. Patent 2,271,623, Carroll and Allen U.S. Patent 2,288,226 and Carroll and Spence U.S. Patent 2,334,864 describe the chemical sensitization of silver halide emulsions with quaternary ammonium compounds.

We have now found that the light sensitivity of silver halide emulsions, with or without optical sensitizing dyes, may be further increased by incorporating in the emulsions certain quaternary dithiocarbamates. These compounds are incorporated in the emulsion after digestion but before coating and exposure. The compounds which we propose to use have the following structure:



in which R represents an alkyl or substituted alkyl group such as methyl, ethyl, propyl, hydroxyethyl, sulfoalkyl or carboxyalkyl, R' represents a lower alkyl group such as methyl or ethyl, x is 1, 2 or 3, and X is an anion or acid radical, for example, halide, p-toluenesulfonate, alkyl sulfate or perchlorate.

The following specific compounds may be employed as sensitizers according to our invention.



2



15

The preparation of silver halide emulsions involves three separate operations: (1) the emulsification and digestion or ripening of the silver halide, (2) the freeing of the emulsion from aqueous soluble salts usually by washing, and (3) the second digestion or after-ripening to obtain increased sensitivity (Mees, "The Theory of the Photographic Process," 1942, page 3). Our sensitizing agents may be added at any stage in the preparation but preferably after the final digestion.

20 The photographic emulsions which we use are of the developing-out type, and best results have been obtained with gelatino-silver bromoiodide emulsions. However, emulsions of varying halide content may be used.

25 The emulsions may be chemically sensitized by any of the accepted procedures, for example, by digestion with naturally active gelatin or the addition of sulfur compounds such as those described in Sheppard U.S. Patents 1,574,944 and 1,623,499 and Sheppard and Brigham U.S. Patent 2,410,689.

30 The emulsions may also be treated with salts of the noble metals such as ruthenium, rhodium, palladium, iridium and platinum, all of which belong to group VIII of the periodic table of elements and have an atomic weight greater than 100. Representative compounds are ammonium chloropalladate, potassium chloroplatinate and sodium chloropalladite, which are used for sensitizing in amounts below that which produces any substantial fog inhibition, as described in Smith and Trivelli U.S. Patent 2,448,060, and as anti-foggants in higher amounts, as described in Trivelli and Smith U.S. Patents 2,566,245 and 2,566,263.

35 The emulsions may also be chemically sensitized with gold salts as described in Waller and Dodd U.S. Patent 2,399,083 or stabilized with gold salts as described in 40 Damschroder U.S. Patent 2,597,856 and Yutzy and Leermakers U.S. Patent 2,597,915. Suitable compounds are potassium chloroaurite, potassium aurithiocyanate, potassium chloroaurate, auric trichloride and 2-aurosulfo-benzothiazole methochloride.

45 The emulsions may also be chemically sensitized with reducing agents such as stannous salts (Carroll U.S. Patent 2,487,850), polyamines such as diethylene triamine (Lowe and Jones U.S. Patent 2,518,698), polyamines such as spermine (Lowe and Allen U.S. Patent 2,521,925), or bis-( $\beta$ -aminoethyl) sulfide and its water-soluble salts (Lowe and Jones U.S. Patent 2,521,926).

50 The emulsions may also be stabilized with the mercury compounds of Allen, Byers and Murray U.S. application Serial No. 319,611, Carroll and Murray U.S. application Serial No. 319,612 and Leubner and Murray U.S. application Serial No. 319,613, all filed November 8, 1952, now U.S. Patents 2,728,663, 2,728,664 and 2,728,665, respectively, granted December 27, 1955.

55 Other stabilizing agents may be added to the emulsions containing the quaternary ammonium compounds and polyalkylene oxides such as cadmium chloride, cadmium

nitrate, cobalt nitrate, manganese chloride, manganese sulfate, zinc chloride, zinc nitrate and zinc sulfate.

The emulsions sensitized with quaternary dithiocarbamates may be additionally sensitized with alkylene oxide polymers or derivatives of alkylene oxides.

The alkylene oxide polymers used to sensitize the emulsions may be of various types. The alkylene oxides from which the polymers are derived contain from 2 to 4 carbon atoms, e.g., ethylene oxide, propylene oxide and butylene oxide. The preparation of polymers from these compounds is described in Ellis, *The Chemistry of Synthetic Resins* (1935), pages 990 to 994. These compounds are also referred to as polyalkylene glycols and their use as sensitizers for silver halide emulsions is described in U.S. Patents 2,423,549 and 2,441,389. The alkylene oxide derivatives may be prepared by condensing an organic compound containing an active hydrogen atom with an alkylene oxide polymer, or by condensing the active hydrogen compound with the alkylene oxide during the polymerization of the latter material.

Various derivatives of alkylene oxides may also be used to sensitize the emulsions, e.g., condensation products of alkylene oxide with organic compounds containing an active hydrogen atom. Examples of "active hydrogen organic compounds," i.e., compounds in which a hydrogen atom may be replaced by reaction of the compound with metallic sodium, methylmagnesium iodide, etc., include alcohols, amines, mercaptans, acids, amides, hydrocarbons such as acetylene, and compounds having the active hydrogen in a methylene group such as dibenzoylmethane. More specifically, we may employ condensation products of alkylene oxide with glycols such as those having from 8 to 18 carbon atoms as described in U.S. Patent 2,240,472 and British Patent 443,559 as well as condensation products of alkylene oxides with aliphatic alcohols, condensation products of alkylene oxides with aliphatic acids, e.g., lauric acid and glycine, condensation products of alkylene oxides with aliphatic amines or amides, e.g., glycine and lauryl amide, and condensation products of alkylene oxides with phenols, e.g., phenol. The preparation of these condensation products is described in U.S. Patent 1,970,578. Condensation products of alkylene oxides with hexitol ring dehydration products as described in U.S. Patent 2,400,532 may also be employed.

Fog in emulsions sensitized with our compounds may be reduced by the use of antifoggants, for example, azaindenes such as the compounds disclosed in *Zeitschrift für Wiss. Phot.*, 47, 2-28 (1952), and in U.S. Patent 2,716,062. However, speed increases are obtained with the quaternary dithiocarbamates in the absence of such antifoggants.

Our invention is further illustrated by reference to the following example:

#### EXAMPLE

To portions of an optically sensitized gelatino-silver bromoiodide emulsion containing about  $\frac{1}{4}$  mol of silver halide per liter, which had been digested with a sulfur compound such as disclosed in Sheppard U.S. Patent 1,574,944, and a gold compound such as disclosed in U.S. Patent 2,399,083, and stabilized with an azaindene, were added the amounts of Compound 5 shown in the following table:

| Compound   | Amount per mole of AgBrI | Relative Speed | Gamma | Fog |
|------------|--------------------------|----------------|-------|-----|
| Control    |                          | 115            | 1.22  | .12 |
| Compound 5 | .75                      | 166            | 1.03  | .16 |
| Compound 5 | 3.0                      | 174            | .96   | .18 |

The emulsions were coated on film support in the conventional manner, exposed on an Eastman-type 1-b sensitometer and processed for 5 minutes in DK-50 developer having the following composition with the results shown

in the table, speed being shown as a relative speed in each case with the control being designated 115:

| Developer DK-50:               | Grams |
|--------------------------------|-------|
| N-methyl-p-aminophenol sulfate | 2.5   |
| Hydroquinone                   | 2.5   |
| Sodium sulfite, desiccated     | 30.0  |
| Sodium metaborate              | 10.0  |
| Potassium bromide              | 0.5   |
| Water to make 1 liter.         |       |

The compounds which we use may be prepared as follows:

#### Compound 5

##### $\gamma$ -3-CHLOROPROPYL PYRIDINE

Thionyl chloride (90 g.) was added dropwise to 68.5 g. of 4-pyridinepropanol in 250 ml. of chloroform over a 25-minute period. When the initial exothermic reaction ceased, the solution was heated at reflux temperature for one hour. The black reaction mixture was poured onto ice, the aqueous layer was made basic to litmus by the addition of 50 percent KOH solution, and after thorough shaking in a separatory funnel, the chloroform layer was removed. The aqueous layer was extracted with 150 ml. of chloroform, and the combined chloroform extracts were decolorized with activated carbon and dried over magnesium sulfate. The volatiles were then removed in vacuo, and the residue was distilled, giving 80-85 percent of  $\gamma$ -3-chloropropylpyridine.

*Analysis.*—Calc'd. for  $C_8H_{10}NCl$ : N, 9.0. Found: N, 9.2.

This compound was stored at  $-20^{\circ}$  to prevent polymerization which occurs slowly at room temperature. Although a larger quantity may be prepared in one experiment, attempts to distill more than about 125 g. at one time resulted in a lower yield and occasionally led to a violent, exothermic polymerization in the distillation flask.

##### 3-( $\gamma$ -PYRIDYL)PROPYL DIMETHYLDITHIOCARBAMATE

To 10.1 g. of sodium dissolved in 500 ml. of dry methanol was added 73 g. of dimethylammonium dimethyldithiocarbamate with stirring. The yellow-to-green solution was treated with 45 g. of  $\gamma$ -3-chloropropylpyridine, and the reaction mixture was heated with stirring for 6.5 hours. The volatiles were removed on the steam bath until the volume of solution was about 250 ml. This boiling residue was treated with activated carbon and filtered. The filtrate was cooled, and 250 ml. of water was added with cooling and scratching of the flask with a glass rod. After standing in the refrigerator overnight, the light brown crystals were filtered and recrystallized from hexane-chloroform solution, yielding 41.5 g. (60 percent) of 3-( $\gamma$ -pyridyl)propyl dimethyldithiocarbamate which melted at 60.5-63°. Further recrystallization from the same solvent afforded an analytical sample, M.P. 62-4°.

*Analysis.*—Calc'd. for  $C_{11}H_{16}N_2S_2$ : C, 55.0; H, 6.7; N, 11.6. Found: C, 55.0; H, 6.7; N, 11.6.

##### $\gamma$ -[3-(DIMETHYLDITHIOCARBAMATO)PROPYL] - N-METHYL PYRIDINIUM p-TOLUENESULFONATE (COMPOUND 5)

To 3.8 g. of 3-( $\gamma$ -pyridyl)propyl dimethyldithiocarbamate in 50 ml. of dry ether was added 3.5 g. of freshly distilled methyl p-toluenesulfonate, and the solution was heated under reflux for 3-6 hours. The precipitate was filtered and twice recrystallized from acetone. The  $\gamma$ -[3-(dimethyldithiocarbamato)propyl] - N-methylpyridinium p-toluenesulfonate thus prepared weighed 4.8 g. (71 percent of the theoretical) and melted at 109.5-11°.

*Analysis.*—Calc'd. for  $C_{19}H_{26}N_2O_3S_3$ : C, 53.6; H, 6.1; N, 6.6; S, 22.5. Found: C, 53.8; H, 6.0; N, 6.7; S, 22.8.

#### Compound 1

##### $\gamma$ -PICOLYL DIMETHYLDITHIOCARBAMATE

By essentially the procedure described above for 3-( $\gamma$ -pyridyl)propyl dimethyldithiocarbamate, using  $\gamma$ -picolyl

chloride hydrochloride,  $\gamma$ -picolyl dimethyldithiocarbamate was prepared. Recrystallization of the crude product from chloroform-hexane solvent pair afforded a pure sample, in 59 percent yield, which melted at 67.5-69°.

*Analysis.*—Calc'd. for  $C_9H_{12}N_2S_2$ : C, 51.0; H, 5.7; N, 12.7. Found: C, 51.4; H, 6.0; N, 12.6.

$\gamma$ -DIMETHYLDITHIOCARBAMATOMETHYL-N-METHYL-PYRIDINIUM p-TOLUENESULFONATE (COMPOUND 1)

This compound, prepared in 80 percent yield as described for Compound 5, melted at 93-4°.

*Analysis.*—Calc'd. for  $C_{17}H_{22}N_2O_3S_3$ : N, 7.0. Found: N, 6.8.

*Compound 2*

$\beta$ -PICOLYL DIMETHYLDITHIOCARBAMATE

This compound was prepared in 68 percent yield from  $\beta$ -picolyl chloride HCl. It is a yellow oil.

*Analysis.*—Calc'd. for  $C_9H_{12}N_2S_2$ : C, 51.0; H, 5.7. Found: C, 51.0; H, 5.5.

$\beta$ -DIMETHYLDITHIOCARBAMATOMETHYL-N-METHYL-PYRIDINIUM p-TOLUENESULFONATE (COMPOUND 2)

This compound was prepared in 87 percent yield as described for Compound 5 and melted at 161-162.5° after recrystallization from methanol-acetone.

*Analysis.*—Calc'd. for  $C_{17}H_{22}N_2O_3S_3$ : C, 51.3; H, 5.6; N, 7.0. Found: C, 51.1; H, 5.9; N, 6.7.

*Compound 3*

3-( $\gamma$ -PYRIDYL)PROPYL DIETHYLDITHIOCARBAMATE

This compound was prepared in 71 percent yield from  $\gamma$ -3-chloropropyl-pyridine and sodium diethyldithiocarbamate. It is a yellow oil, B<sub>0.2</sub> 177°, which was further purified by chromatography using alumina.

*Analysis.*—Calc'd. for  $C_{13}H_{20}N_2S_2$ : C, 58.1; H, 7.5; N, 10.4. Found: C, 58.2; H, 7.2; N, 10.0.

$\gamma$ -[3-(DIETHYLDITHIOCARBAMATO)PROPYL]-N-METHYL-PYRIDINIUM PERCHLORATE (COMPOUND 3)

The p-toluenesulfonate salt, prepared in the usual manner, was so hygroscopic that a water solution of it was treated with an excess of sodium perchlorate in water. The non-hydroscopic perchlorate salt (73 percent yield) was filtered and recrystallized three times from acetone-water solvent pair to afford a pure sample of the title compound which melted at 101-2°.

*Analysis.*—Calc'd. for  $C_{14}H_{23}ClN_2O_4S_2$ : N, 7.3; S, 16.7. Found: N, 7.2; S, 16.6.

*Compound 4*

3- $\beta$ -PYRIDYLPROPYL DIMETHYLDITHIOCARBAMATE

$\beta$ -3-Chloropropylpyridine was prepared from 3-pyridine-propanol by the method described for Compound 5. The  $\beta$ -3-chloropropylpyridine was then reacted with dimethylammonium dimethyldithiocarbamate as described for Compound 5. However, the product did not crystallize but was isolated as an oil. This brown oil was further purified by chromatography using alumina as the adsorbent and ether as the solvent. A light yellow oil resulted.

*Analysis.*—Calc'd. for  $C_{11}H_{16}N_2S_2$ : C, 55.0; H, 6.7. Found: C, 55.0; H, 7.1.

$\beta$ -[3-(DIMETHYLDITHIOCARBAMATO)PROPYL]-N-METHYL-PYRIDINIUM PERCHLORATE (COMPOUND 4)

The p-toluenesulfonate salt, obtained by heating methyl p-toluenesulfonate and 3- $\beta$ -pyridylpropyl dimethyldithiocarbamate together in ether, was treated with a water solution of sodium perchlorate. The resulting white solid was filtered and recrystallized, from acetone-water solvent pair and then from acetone giving the title compound, melting at 75-76.5° in 50 percent yield.

*Analysis.*—Calc'd. for  $C_{12}H_{19}ClN_2O_4S_2$ : N, 7.9; S, 18.0. Found: N, 7.7; S, 18.3.

The sensitivity increase produced by the quaternary dithiocarbamates is unexpected for a number of reasons. In the first place, they contain the thiocarbonyl group  $=C=S$  which is usually an active source of desensitiza-

tion. Furthermore, they are of relatively low molecular weight compared to many of the prior sensitizers. Without the quaternary nitrogen atom, these compounds would be incapable of increasing the sensitivity of an already fully chemically sensitized emulsion. Both sulfur atoms in the compound are necessary for activity, and the reversal of the



in the chain destroys their activity.

The chemical sensitizing agents and other addenda which we have described may be used in various kinds of photographic emulsions. In addition to being useful in non-optically sensitized emulsions they may also be used in orthochromatic, panchromatic and X-ray emulsions. They may be added to the emulsion before or after any sensitizing dyes which are used. Various silver salts may be used as the sensitive salt such as silver bromide, silver iodide, silver chloride or mixed silver halides such as silver chlorobromide or silver bromoiodide. The agents may be used in emulsions intended for color photography, for example, emulsions containing color-forming couplers or emulsions to be developed by solutions containing couplers.

The dispersing agent for the silver halide may be gelatin or other colloidal material such as collodion, albumin, cellulose derivatives or synthetic resins.

It will be understood that we contemplate as included 30 within our invention all modifications and equivalents falling within the scope of the appended claims.

What we claim is:

1. A light-sensitive silver halide emulsion sensitized with a quaternary dithiocarbamate having the following 35 composition:



40 in which R is selected from the class consisting of lower alkyl, hydroxy lower alkyl and carboxy lower alkyl groups, R' represents a lower alkyl group, x is an integer from 1 to 3, and X represents an anion.

2. A light-sensitive silver halide emulsion sensitized 45 with a quaternary dithiocarbamate having the following composition:



50 in which x is an integer from 1 to 3, and X is selected from the group consisting of perchlorate and p-tolene sulfonate.

3. A light-sensitive silver halide emulsion sensitized 55 with a quaternary dithiocarbamate having the following composition:



60 in which x is an integer from 1 to 3, and X is selected from the group consisting of perchlorate and p-tolene sulfonate.

4. A light-sensitive silver halide emulsion sensitized 65 with a quaternary dithiocarbamate having the following composition:



References Cited in the file of this patent

FOREIGN PATENTS